

## UNITED STATES PATENT OFFICE

2,406,667

MOTOR FUELS AND PROCESSES FOR  
MAKING SAME

Louis A. Clarke, Fishkill, N. Y., assignor to The  
Texas Company, New York, N. Y., a corporation  
of Delaware

No Drawing. Original application July 23, 1942,  
Serial No. 452,061. Divided and this applica-  
tion April 27, 1943, Serial No. 484,765

3 Claims. (Cl. 44—80)

1

My invention relates to improved fuels for internal combustion engines, and to methods for producing and utilizing such fuels.

In the past, motor fuels have generally been rated on the basis of their performance under relatively lean mixture operating conditions. This has resulted from considerations of fuel economy in the operation of automotive engines, and test methods such as the CFR octane number determinations have been devised accordingly. Moreover, most fuels have somewhat better anti-knock characteristics under rich mixture operating conditions, i. e., air-fuel ratios of about 12/1, than under lean mixture operating conditions, i. e., air-fuel ratios of about 15/1. In the usual automotive engine, air-fuel ratios of less than 12/1 have been of no interest, since the use of such mixtures has resulted in both loss of power and loss of economy.

In the operation of supercharged engines, on the other hand, and especially those of high speed, high heat load types, the performance of fuels in mixtures richer than 12/1 becomes important. With such engines, the maximum power output at full throttle, without detonation, is obtainable only with super-rich mixtures, i. e., with air-fuel ratios less than 11/1, and usually considerably below 10/1. In order to obtain maximum power output from an aircraft engine for take-off under heavy load, it is desirable to employ a fuel having anti-knock characteristics especially suited for operation at such super-rich mixtures.

It has been found that various fuels differ markedly in their performance in super-rich mixture, even though their anti-knock characteristics at leaner mixtures may be substantially identical. Certain of the aromatic hydrocarbons such as benzene and toluene, when incorporated in a motor fuel, have been found to have the characteristic of considerably improving the fuel in its performance in super-rich mixtures, although often at a considerable sacrifice of lean mixture performance. On the other hand, the aliphatic hydrocarbon anti-knock standard, 2,2,4-trimethylpentane, does not have this property of preferentially improving the super-rich mixture performance of base fuels to which it is added; and the paraffin hydrocarbons have generally been recognized to be lacking in the desired superior performance in super-rich mixtures.

I have now found, however, that 2,3-dimethylbutane possesses outstanding anti-knock characteristics in operation at air-fuel ratios of less than 11/1, and is especially useful in the formulation

2

of "super fuels" for use in supercharged aircraft engines. The performance of 2,3-dimethylbutane in fuels at super-rich mixtures is greatly superior to the performance of other aliphatic hydrocarbons such as "isooctane," and is unexpectedly much superior to the performance of its closest isomer, 2,2-dimethylbutane. I have further found that this improvement in super-rich mixture performance may be obtained by the use of 2,3-dimethylbutane without a simultaneous loss in lean mixture performance of the degree encountered when employing aromatic hydrocarbons for this purpose.

Since 2,3-dimethylbutane is very satisfactory for both lean and super-rich mixture operation, a fuel comprising essentially this hydrocarbon could be employed for all purposes. However, additional fuel constituents of higher and lower volatility than 2,3-dimethylbutane will usually be desirable for the production of a balanced fuel. Furthermore, for economic reasons it will usually not be desirable to employ a fuel consisting essentially of 2,3-dimethylbutane, since satisfactory performance can usually be obtained by the use of some what less expensive fuel stocks in conjunction with 2,3-dimethylbutane. Fuels comprising essentially 2,3-dimethylbutane will, therefore, be of most value as auxiliary fuels, to be blended with, or to be employed in conjunction with, other fuels which do not have satisfactory performance in super-rich mixtures.

As an auxiliary fuel, 2,3-dimethylbutane, or a solution having a relatively high concentration of 2,3-dimethylbutane, may be substituted for the primary fuel for operation at maximum power output, or may be blended with the primary fuel at times of increased power demands on the engine. In the former case, the fuel supply may suitably be changed manually, as in changing from a take-off fuel to a cruising fuel in aircraft operation. Where the auxiliary fuel is to be blended with the main fuel at times of increased power demand on the engine, this is preferably accomplished by an automatic blending device such as that described in U. S. Patent 2,002,482 of Leo B. Kimball. Other equivalent methods for employing the auxiliary fuel may also be used, such as supplying it to an auxiliary carburetor jet with functions only at full throttle. In any case, the air-fuel ratio should be manually or automatically reduced to a value below 11/1 when the auxiliary fuel is supplied to the engine, in order to obtain increased power output.

Although it will usually be most economical to employ 2,3-dimethylbutane as an auxiliary fuel

only at times of increased power demands on the engine, it will often be most practical to employ only a single fuel having satisfactory anti-knock characteristics in both lean mixtures and super-rich mixtures. For this purpose, a base fuel is chosen which has satisfactory performance in lean mixtures, and 2,3-dimethylbutane is incorporated in the fuel in an amount sufficient to improve the performance of the fuel in super-rich mixtures. Any amount which produces a measurable improvement may be employed, but I usually prefer to use at least 10% by volume, and preferably 20-30% or more, depending upon the anti-knock characteristics of the base fuel, and on the character and amount of any additional anti-knock agents employed.

The base fuels with which 2,3-dimethylbutane may be employed, either in blended mixtures or in separate auxiliary fuels, may be any of the known types of motor fuels for internal combustion engines. Straight run gasolines, thermally or catalytically cracked gasolines, polymer gasolines, alkylation gasolines, thermally or catalytically reformed or hydroformed gasolines, and various blends of such products are suitable for the present purpose. Base fuels which are especially desirable are those having high power output in lean mixtures, such as fuels containing relatively large amounts of 2,2,4-trimethylpentane. The alkylate from the hydrogen fluoride alkylation of isobutane with isobutylene, as described in my co-pending application, Ser. No. 429,471, filed February 4, 1942, and the hydrogenated dimer from the cold acid polymerization of isobutylene, are especially suited for this purpose.

The base fuels and auxiliary fuels, or the blended fuels, may all contain additional anti-knock additives and other common fuel constituents such as gum inhibitors, agents for scavenging metallic engine deposits, and the like. The anti-knock properties of 2,3-dimethylbutane in super-rich mixtures are especially advantageous in fuels containing other anti-knock components. Although different types of anti-knock materials in admixture often produce much less than additive results, the preferential improvement in super-rich mixtures produced by 2,3-dimethylbutane appears to be at least additive with the effects of other anti-knock components such as tetra-ethyl lead. It is to be understood, therefore, that one aspect of my invention constitutes the use of 2,3-dimethylbutane in conjunction with any of the known anti-knock additives such as tetra-ethyl lead, iron pentacarbonyl, aromatic hydrocarbons, or aromatic amines.

Although various chemical syntheses may be employed for the production of 2,3-dimethylbutane, one of the most economic sources is the alkylation of isobutane with ethylene, using an aluminum halide catalyst as disclosed in my co-pending application Ser. No. 439,299, filed April 17, 1942. The pure compound, 2,3-dimethylbutane, may be recovered from such alkylation products by fractional distillation, if desired. However, the over-all alkylate, or a relatively wide-boiling cut containing 2,3-dimethylbutane, may be used as the auxiliary fuel in the present invention, or for blending with other base fuels to improve their performance in super-rich mixtures.

The rich mixture performance of 2,3-dimethylbutane is illustrated in the following examples:

## Example I

A supercharged test engine was employed to test the power output of a fuel consisting of 2,3-dimethylbutane plus 3 ml. of tetra-ethyl lead per gallon, in accordance with the AFD-3C test method. At an air-fuel ratio of approximately 10.5/1 the permissible indicated mean effective pressure (IMEP without detonation) was 259 lbs./sq. in. This corresponded to the maximum power output which could be absorbed by the test engine dynamometer, but the trend of the measured values of IMEP indicated that the fuel would be capable of much greater power output in still richer mixtures. In a comparable test in the same engine, commercial 2,2,4-trimethylpentane plus 6 ml. of tetra-ethyl lead per gallon produced a permissible IMEP of only approximately 221 lbs./sq. in. at an air-fuel ratio of 10.5/1 and a maximum permissible IMEP of only 249 lbs./sq. in. at an air-fuel ratio of approximately 8/1.

## Example II

A fuel consisting of 75% by volume of commercial 2,2,4-trimethylpentane and 25% by volume of 2,3-dimethylbutane, plus 3 ml. of tetra-ethyl lead per gallon, was tested by the AFD-3C method. The maximum permissible IMEP was found to be 243 lbs./sq. in. at an air-fuel ratio of approximately 10.5/1. In a comparable test in the same engine, commercial 2,2,4-trimethylpentane plus 4 ml. of tetra-ethyl lead per gallon gave a maximum permissible IMEP of only 233 lbs./sq. in.

## Example III

A fuel consisting of 80% by volume of a debutanized 300° F. end-point alkylation gasoline (from the sulfuric acid alkylation of isobutane with butylenes) and 20% by volume of 2,3-dimethylbutane, plus 3 ml. of tetra-ethyl lead per gallon, was tested by the AFD-3C method. The maximum permissible IMEP was found to be 218 lbs./sq. in. at an air-fuel ratio of approximately 8.5/1, as compared to a maximum permissible IMEP for 100% debutanized alkylate, plus 3 ml. of tetra-ethyl lead, of only approximately 195 lbs./sq. in. At a lean mixture (air-fuel ratio of approximately 14.3/1) the permissible IMEP values for these two fuels were 111 lbs./sq. in. and 95 lbs./sq. in., respectively.

Comparable tests with the same alkylation gasoline, leaded to the extent of 4 ml. of tetra-ethyl lead per gallon, with and without ethylbenzene for improving the super-rich mixture performance, are shown in the table below:

| Fuel composition       | Max. IMEP, lbs./sq. in. | Change in max. IMEP | Lean IMEP (fuel/air = 0.07) | Change in lean IMEP |
|------------------------|-------------------------|---------------------|-----------------------------|---------------------|
| 100% 300° alkylate     | 195                     |                     | 95                          |                     |
| 3.0 ml. TEL/gal.       |                         |                     |                             |                     |
| 80% 300° alkylate      | 218                     | +23                 | 111                         | +16                 |
| 20% 2,3-dimethylbutane |                         |                     |                             |                     |
| 3.0 ml. TEL/gal.       |                         |                     |                             |                     |
| 100% 300° alkylate     | 206                     |                     | 106                         |                     |
| 4.0 ml. TEL/gal.       |                         |                     |                             |                     |
| 80% 300° alkylate      | 227                     | +21                 | 97                          | -9                  |
| 20% ethylbenzene       |                         |                     |                             |                     |
| 4.0 ml. TEL/gal.       |                         |                     |                             |                     |

As may be seen from the above table, 2,3-dimethylbutane is superior to ethylbenzene for improving the performance of this alkylation gasoline in super-rich mixtures without sacrificing lean mixture performance.

This application is a division of application of

Louis A. Clarke, Serial No. 452,061, filed July 23, 1942, for "Motor fuels and processes for making and utilizing same." Said application Serial No. 452,061 is a continuation-in-part of application of Louis A. Clarke, Serial No. 439,299, filed April 17, 1942, which in turn is a continuation-in-part of applications, Serial No. 324,784, filed March 19, 1940 and Serial No. 327,575, filed April 3, 1940.

It is to be understood, of course, that the above examples are merely illustrative, and do not limit the scope of my invention. As has previously been pointed out, other constituents may be employed in blended fuels containing 2,3-dimethylbutane, and such fuels may be formulated in accordance with prior practices in the art, except for the improvement in super-rich mixture operation effected by the incorporation of 2,3-dimethylbutane. It should also be understood that 2,3-dimethylbutane is especially adapted for use in conjunction with all other types of anti-knock additives such as aromatic hydrocarbons, aromatic amines, and other organo-metallic anti-knock agents, as well as the particular materials employed in these examples. In general, it may be said that the use of any equivalents, or modifications of procedure which would naturally occur to those skilled in the art, is included in the scope of this invention. Only such limitations as are indicated in the appended claims should be imposed on the scope of my invention.

I claim:

1. An aviation fuel blend adapted for use in supercharged engines and having a preferentially improved maximum power output at full throttle, without detonation, at super-rich air-fuel ratios richer than 11:1, as compared with lean air-fuel ratios leaner than 11:1, comprising a high anti-knock rating base fuel containing a major proportion of isoparaffinic hydrocarbons and an anti-knock additive, and a blending fuel comprising

40

2,3-dimethylbutane in major proportion by volume of the blending fuel, the latter being added in sufficient proportion to include at least 10%-30% by volume of 2,3-dimethylbutane in the base fuel and sufficient to convert the base fuel into the aforesaid aviation fuel blend.

2. An aviation fuel blend adapted for use in supercharged engines and having a preferentially improved maximum power output at full throttle, without detonation, at super-rich air-fuel ratios richer than 11:1, as compared with lean air-fuel ratios leaner than 11:1, comprising a high anti-knock rating base fuel containing a major proportion of isobutane-butylene alkylate gasoline and an anti-knock additive, and a blending fuel comprising 2,3-dimethylbutane in major proportion by volume of the blending fuel, the latter being added in a proportion to include at least 10%-30% by volume of 2,3-dimethylbutane in the base fuel and sufficient to convert the base fuel into the aforesaid aviation fuel blend.

3. An aviation fuel blend adapted for use in supercharged engines and having a preferentially improved maximum power output at full throttle, without detonation, at super-rich air-fuel ratios richer than 11:1, as compared with lean air-fuel ratios leaner than 11:1, comprising a high anti-knock rating base fuel consisting essentially of a debutanized aviation fraction of alkylation acid catalyzed isobutane-butylene alkylate and an anti-knock additive, and a blending fuel consisting essentially of a wide-boiling cut of aluminum chloride catalyzed isobutane-ethylene alkylate containing a major proportion by volume of 2,3-dimethylbutane, said blending fuel being added in a proportion to include at least 10%-30% by volume of 2,3-dimethylbutane in the base fuel and sufficient to convert the base fuel into the aforesaid aviation fuel blend.

LOUIS A. CLARKE.